# EUROPEAN PATENT APPLICATION

(11) **EP 0 493 026 A2**
(43) Date of publication of application: **01.07.1992**
(21) Application number: 91311881.6
(22) Date of filing: 20.12.1991
(51) Int. Cl.: A24D 3/14, A24D 3/10

(54) **Cigarette filter**

(30) Priority: 25.12.1990 SU 4896031
(71) Applicant: Voronkov, Mikhail Grigorievich, Irkutsk (SU); Sinelnikov, Leonid Yakovlevich, Moscow (SU); Vlasova, Natalya Nikolaevna, Irkutsk (SU); Kaplan, Elizar Yakovlevich, Moscow (SU); Pestunovich, Antonina Egorovna, Irkutsk (SU); Safaev, Radzhab Davronovich, Moscow (SU); Belitsky, Gennady Alterovich, Moscow (SU)
(72) Inventor: Voronkov, Mikhail Grigorievich, Irkutsk (SU); Sinelnikov, Leonid Yakovlevich, Moscow (SU); Vlasova, Natalya Nikolaevna, Irkutsk (SU); Kaplan, Elizar Yakovlevich, Moscow (SU); Pestunovich, Antonina Egorovna, Irkutsk (SU); Safaev, Radzhab Davronovich, Moscow (SU); Belitsky, Gennady Alterovich, Moscow (SU)
(74) Representative: Bibby, William Mark

(57) **Abstract**

A cigarette filter comprises a base made of acetate, cellulose or acetate-cellulose fibers and impregnated with an adsorbing, agent which is a N,N′-bis(3-triethoxysilylpropyl)thiocarbamide organo-silicon monomer (C₂H₅O)₃Si(CH₂)₃NH - C(S) -NH(CH₂)₃Si-(OC₂H₅)₃.

## Description

### Field of the invention

The present invention relates to techniques for purifying tobacco smoke of cancerogenic and toxic substances and in particular to a cigarette filter. The filter ran be used in the tobacco industry in manufacturing filter cigarettes.

### Backround of the Invention

Known in the art are filters comprising a base charcoal of acetate-cellulose fibers in combination with charcoal. The charcoal is containing in the base, as mechanical inclusions, and forming a coat of the base or simply contacting it. These filters are deficient in that they do not completely eliminate a harmful effect of a number of the cancerogenic and toxic components of tobacco smoke.

In this connection effective filtration means are needed which remove, if possible, the great amounts of tobacco smoke harmful components, but permit preserving its organoleptic characteristics.

Also known is another cigarette filter made from hydroxyapatite in combination with acetate fibers or activated coal. Said hydroxyapatite may be represented by the formula 3[Ca₃(PO₄)₂] M (OH)₂. It is substantially a material having a particle size of from 2 to 5µm and used in the filter in an amount of from 0, 1 to 20% of the tobacco weight in the cigarette. This filter can be made in the form of a tablet, sleeve, mouthpiece and etc. The filter contributes to an improved absorption of harmful substances from the tobacco smoke, such as nicotine, tar, carbon mono oxide. It does not promote, however, to absorbing cancerogenic and toxic substances, from tobacco smoke such as polycyclic aromatic hydrocarbons benz (a) pyrene, benz (g,h,i) perylene, dibenz(a,h) anthracene, dihenz (a,c) anthracene and volatile nitrosoamines (N′- -nitrosodiethylamine,N′-nitrosopyrrolidine).
There are known various cigarette filters which decrease a toxic effect of tobacco smoke and consist of a base made of acetate, cellulose on acetate-cellulose fibers with substances applied onto the base which having absorption properties or impregnated with these substances.

The adsorbing agents used are represented by activated charcoal, the inorganic and organic salts of mercaptoalkanesulfonic acids (cysteine, acetylcysteine and phthalocyanins).

These filters are deficient in that the range of substances absorbed by them is restricted in all cases, while the very filters can degrade on heating with the formation of toxic compounds. For instance, employment of phthalocyanine as a sorbent may result in forming the following products of decomposition: organic cyanides, ammonia, benzene derivatives etc.

Closest to the claiemd filter is one (ref.publication No. 0351252, dated January 17, 1990, of European Patent Application No.89307209.0) containing a base made of acetate, cellulose or acetate-cellulose fibers, and impregnated with an absorbin agent which is a complex compound of ferrous iron with a ligand being in reality a thiol-containing low molecular compound in which a ratio of iron ions to the number of ligand molecules not more than 1:2 and a proportion of the absorbing agent is between 3 and 13% of the total weight of the filter.

In the filter as described the sources of obtaining ferrous iron usually were the salts of iron, for example, FeSO₄, FeCl₂, Fe(NO₃)₂, and as the thiol-containing low- -molecular compounds were used monothiol-containing compounds (thiol-sulphate of sodium, cysteine, reduced glutathione etc) and dithiol-containing organic compounds (diethyldithiocarbamate, dimethyldithiocarbamate, ethyl-xanthate of sodium etc).

The filter as described enables one to efficiently clean tobacco smoke from nitrogen oxide, but is does not raise, just as all the filters described earlier, the content in the tobacco smoke such cancerogenic and toxic substances as polycyclic aromatic hydrocarbons (benz(a ) pyrene, benz(g, h,i) perylene, dibenz(a,h) anthracene, dibenz(a,c) anthracene), volatile nitrosoamines (N′-nitrosodiethylamine, N′-nirosopyrrolidine) as well as metals, such as magnesium, calcium, strontium, copper, lead, arsenic, vanadium, chromium, manganese, iron, cobalt and nickel.

### Summery of the Invention

An object of the present invention is to raise the degree of purificaiton of tobacco smoke of cancerogenic and toxic substances.

Said object is achieved by a cigarette filter comprising a base of acetate, cellulose of acetate-cellulose fibers impregnated with an adsorbing agent. According to the invention, the adsorbing agent used is represented by an N,N′-bis(3-thriethoxysilylpropyl)thiocarbamide organo--silicon monomer (C₂H₅O)₃Si(CH₂)₃NH-C(S)-NH(CH₂)₃ Si(OC₂H₅)₃.

The filter as claimed provides for the 100% removal of polycyclic aromatic hydrocarbons, of about 60% of volatile nitrosoamines and up to 90% of metals owing to the employment of the adsorbing agent as proposed. The content of adsorbing agent should preferably be from 6 to 15,3% of the weight of the base fibers, a factor that assures the maximal efficiently of purification of tobacco smoke from cancerogenic and toxic agents.

### Detailed Description of the Invention

The invention is further explained by a description of its specific embodiments.

A cigarette filter comprises a base of acetate, cellulose or acetate-cellulose fibers, impregnated with an adsorbing, agent which is an N,N′-bis(3-thriethoxysilylpropyl)thiocarbamide organo-silicon monomer (C₂H₅O)₃Si(CH₂)₃NH-C(S)-NH(CH₂)₃Si(OC₂H₅)₃.

The content of said monomer in the filter is from 6 to 15,3% of the weight of the base fibers.. With the content of the monomer of less than 6% the base fiber proves to be insufficiently impregnated with this monomer, and its adsorption properties get worse. With the content of the monomer more than 15,3% its quantity proves to be excessive, and a certain amount of the monomer penetrates into the tobacco of a cigarette and deteriorate its quality.

A mechanism of binding a monoser with the material of a filter base is based on a chemical modification of acetate, cellulose or acetate-cellulose fibers of the base due to the condensation of reactive surface groups (hydroxylic ones, in particular) of said monomer. Condensation is carried out in a way similar to the known modification of a silica gel of various brands according to the possible scheme as follows:

During this process on the surface of acetate, cellulose of acetate-cellulose base fibers there is formed a layer of a polysiloxane polymer which is chemically bound therewith and has effective adsorption properties.

The high sorbtion activity of the monomer for nitrosocompounds and polycyclic aromatic hydrocarbons is explained by the presence therein of reaction centres, as a siloxane base, thiocarbonyl groups and aminogroups, each of them is capable of the chemosorbtion of the cancerogenic or toxic elements of tobacco smoke.

The effective absorption of metals is explained by the complex formation of metals with a pair of active groups of the monomer which contain the atoms of sulfur and nitrogen according to the possible scheme as given below:

In the case of sorbtion of metals whose nature depends on ion bonds, a process fo sorbtion proceeds according to the following scheme

This process is characteristic, for instance in the sorbtion of lead and arsenic which, on the example of lead, process according to the following scheme:

The filter as described above is manfuactured in the following way.

A base of acetate, cellulose or acetate-cellulose fibers is impregnated with 4 to 10% of a solution of the above-identified organo-silicon monomer in an organic solvent and dried.

Following below are the specific examples illustrating a process of manufacturing the filter claimed.

### Example I

A 4% solution of a monomer is prepared in ethyl alcohol, and the solution obtained in an amount of no less than 13 ml is used to impregnate the base of a filter made of acetate fibers in the form of a cylinder having a diameter of 7,9 mm, a lenght of 15 mm and a weight of 110 mg. The resulting base is then dried, and along with this, the weight of the monomer is 6% of the weight of acetate fibers. During drying the monomer is polymerized and bonded with said base acetate fibers.

### Example 2

A 7% solution of a monomer is prepared in ethylalcohol. The obtained solution 13 ml is used for impregnating the base of a filter which is made from acetate-cellulose fibers in the form of a cylinder having a diameter of 7,9 mm, a length of 18 mm, and weight of 137 mg whereupon the resulting base is dried and polymerization takes place of the monomer during drying and its binding with the acetate-cellulose fibers of the base, and along with this, the weight of the monomer is 10,7% of the weight of the said base acetate-cellulose fibers.

### Example 3

A 10% solution of a monomer is prepared in ethyl alcohol. The obtained solution is used in an amount of 13 ml for impregnating the base of the filter which is made from cellulose fibers in the form of a cylinder, having a diameter of 7,9 mm, a lenght of 18 mm and a weight of 130 mg.

The obtained base is then dried, and during drying the monomer is polymerized and bound with the cellulose fibers of the base. The weight of the monomer is 15% of the cellulose fibers of the base.

Cigarettes with the above-described filters were tested according to the following manner.

Prior to analysis, all the cigarettes were conditioned during 48 hours, at 22°C and with a relative humidity of about 60%. They were smoked on a 20-position rotor smoking machine RM20 / CS(Germany "Borgwaldt"), according with the methods given in the "International Standards Organization ISO 3308.
"Cigarettes - Routine analytical cigarette smoking machine. Definitions and standard conditions", Geneva, 1986, P.6.

The volume of puff was 35 ml, duration--2 seconds, frequency--I puff per minute on I Cambridge filter.

The analysis of the contained polycyclic aromatic hydrocarbons in a tobacco smoke condensate was performed according to the modified methods as described in the publication by A.Ya.Khesin et al. "Vozmozhnost kolichestvennogo opredeleniya politsiklicheskikh aromaticheskikh uglevodorodov v zagryazneniyakh okrouzayushchei cheloveka sredy na osnove kvazilineichatykh spektrov lyuministsentsii i vozbouzhdeniya". The journal of aplied spectroscopy, 1983, XXXV111, N 6, pp.922-933. The condensate of tobacco smoke of 10 cigarettes smoked on one Cambridge filter having the dia meter . of 92 mm was extracted with benzene on an ultrasound bath, 60 watt, 30 minutes, twice, and evaporated on a rotor evaporator up to 5 ml, at 35°C. Further, I ml extract was fractionated with the aid of thin layer chromatography with a non-attached thin layer of aluminium oxide in a hexane benzene system with their ration of 3:1. The composition of polycyclic aromatic hydrocarbons was analyzed by registering a quasiline spectrum of fluorescence with the selective excitation of hydrocarbons on a spectrofluorimeter "HITACHI," Japan at a temperature of liquid nitrogen.

The content of metals in the condensate of tobacco smoke was determined according to the modified method set out in the publication by Westcolt D., Sprincer D.

"The cadmium, nickel and lead content of tobacco and cigarette smoke" Beifr. Tabakporsch, 1974, v.7, N 4, pp.217-221, Jenkins R. "Occurrence of selected metals in cigarette tobacco and smoke. Environmental carcinogens selected methods of analysis", Lyon, 1986, IARC Sci. Publ. No.71, v.8, pp.129-138.

More, the atomic-absorption method has been replaced with a plasma emission one. Analysis was performed on a plasma emissive JV-48 spectrometer (Jobin-Ivon, France) with the use of a Cambridge filter having a diameter of 44 mm through which five cigarettes were smoked.

The contained volatile N′-nitrosoamines, N′-nitrosodiethylamine and N′-nitrosopyrrolidine were strictly determined according to the methods as described in the monograph of the International agency of research of cancer IARC. Scientific publications No.45. Environmental carcinogens selected methods of analysis. Vo.6, N-Nitrozo Compounds", Lyon, 1986, pp.69-103.

The resuls of the above-described investigations are tabulated (Tables 1,2,3). Data contained in these tables are average data for the filters having a base made of acetate, cellulose or acetate cellulose fibers. In these tables a control cigarette is a cigarette with a filter, having a base non-impregnated with the claimed monomer.

From inspection of Tables 1,2,3 the claimed filter permits efficiently catching such cancerogenic and toxic agents from tobacco smoke as polycyclic aromatic hydrocarbons, volatile nitrosoamines and metals. Also, the organosilicon monomer utilized in the given filter as an adsorbing agent is non-toxic, the bases impregnated with this monomer are stable in time and retain their properties on heating up to 240°C.

## Claims

1. A cigarette filter comprising a base made of acetate, cellulose or acetate-cellulose fibers and impregnated with an adorbing agent, characterized in that the adsorbing agent used is a N,N′-bis(3-thriethoxysilylpropyl)thiocarbamide organo-silicon monomer (C₂H₅O)₃Si(CH₂)₃NH-C(S)--NH(CH₂)₃Si(OC₂H₅)₃.

2. A filter according to Claim I, characterized in that the content of the adsorbing agent is from 6 to 15,3% of the weight of the base.
